

Mar. 6, 1923.

1,447,817.

J. M. PERRY,  
ART OF CASTING METALS,  
FILED NOV. 16, 1922.

FIG. 1.



FIG. 2.



FIG. 3.



FIG. 4.



FIG. 5.



James M. Perry,  
Inventor

By Horace G. Seitz  
Attorney

## UNITED STATES PATENT OFFICE.

JAMES M. PERRY, OF DETROIT, MICHIGAN, ASSIGNOR OF TWO-THIRDS TO HIMSELF  
AND ONE-THIRD TO HORACE G. SEITZ, OF DETROIT, MICHIGAN.

## ART OF CASTING METALS.

Application filed November 16, 1922. Serial No. 601,351.

*To all whom it may concern:*

Be it known that I, JAMES M. PERRY, a citizen of the United States, residing at Detroit, in the county of Wayne and State of Michigan, have invented certain new and useful Improvements in the Art of Casting Metals, of which the following is a specification.

This invention relates to improvements in the art of casting metals, and pertains more particularly to methods designed to eliminate the presence of imperfections in the casting, such, for instance, as are usually caused by the presence of air or gas bubbles or holes produced by sand particles where the casting is made in sand molds.

One of the major difficulties in producing castings is that caused by the rapid chilling or solidification of the molten metal, especially where the castings are of the thin-walled type. In order that the casting may be of proper character it is essential that the metal be poured with sufficient rapidity that there be no opportunity for one portion—the part into which the initial metal first flows to its final position, for instance—to reach solidification before the remainder of the metal has been poured; this to prevent the formation of specific zonal conditions within the casting. Where metal molds are employed, it may be possible to resist this action by heating the walls of the mold, but where the mold is of sand, this aid cannot be had and the pouring of the metal must be sufficiently rapid to prevent conditions of this kind appearing.

Rapid pouring of the metal raises the problem of the escape of air or gas to prevent the formation of holes in the casting—rendering the casting more or less porous. This is due to the fact that the flow of the metal may imprison bubbles, and these must escape by passing upwardly; and where solidification begins before a bubble has reached the top, it remains imprisoned within the casting and provides an imperfection therein in the form of a hole which may or may not extend to the surface—it is generally found beneath the surface of the casting. And where the casting is had with sand molds, the additional problem arises through the dislodgment of sand particles which pass into the molten metal and must, to be eliminated, rise to the top surface of the casting; should the particle fail to reach

the top, it forms an imperfection which, if exposed by machining, etc., leaves a hole in the casting.

As will be understood, the difficulty in both cases arises by reason of the time element that is introduced through the conditions of the beginning of solidification of the molten metal; whatever that length of time may be, the air or gas bubbles or the sand particles or both must reach the "neck" or other waste portion of the casting before the solidification begins if imperfections of this kind are to be prevented. Where the metal remains fluid or molten sufficiently long, these sources of imperfections will reach the waste zone of the casting—the difficulty comes under conditions where the castings are of such character as to set up the beginning of solidification before the time required for the natural movement of the sources of imperfections has ended.

The problem is one that pertains generally to the art of casting, and becomes of especial importance in connection with comparatively thin-walled structures in which the length of the casting in the vertical direction during pouring is such as to prevent a material distance for the imperfection sources to travel in reaching the waste zone, a condition that tends to produce the gas bubble imperfection due to the necessity for comparatively rapid pouring of the metal. Castings of this kind are required in many arts and have many different cross-sectional shapes, a condition that the present invention is designed to meet.

For the purpose of illustrating the characteristics of the invention, without, however, limiting the same to the particular form and purpose indicated, I disclose herein the application of the invention to the production of castings used for the purpose of a blank from which piston rings are formed, the general method for producing such rings being the formation of a cast cylinder of the proper metal—cast in sand molds—the cylinder being of proper diameter, with comparatively thin walls, and generally of a supply length of about eight inches with the upper end in the form of a "neck" or other type of waste zone; this latter forms a part of the casting and is removed and cast aside during the production of the rings.

Due to the thin walls and the vertical length of the casting, imperfections of the

60

65

70

75

80

85

90

95

100

105

110

type mentioned are generally found in these castings, the number and location of the imperfections varying with different castings, it being an extreme exception to find a cylinder free from all imperfections having these sources. The effect of the presence of these and the effect produced in the cost of piston ring construction can be understood from a brief reference to the construction of the rings from the cylindrical casting or blank.

After casting, the blank is machined to the proper dimensions and cut to produce the proper width of ring. In many forms of rings the cross-section is of a type that does not include parallel walls extending normal to the axis of the blank, and in these cases the machining and production of one ring serves to produce a portion of another ring. The result is that it becomes necessary—to obtain the maximum number of rings from the blank, to machine the latter as if it were wholly free from imperfections, after which the rings are inspected, and those found imperfect are cast aside as not usable; since the rings are of narrow width, the dividing of the blank serves to practically expose—at some point at least—the presence of the hole or depression that stamps the ring as a discard.

From this it is possible to see that the presence of the imperfections involves considerably more than the simple loss of the material found in the immediate zone of the imperfection. Whether or not the ring be a perfect ring or a discard, the machining and other production cost is the same in each case—whatever be the cost of the perfect ring, the same cost applies to the discard. Not only is this excess loss present—due to the necessity for completing the discard the same as if it be a perfect ring—another additional cost is found in the necessity for inspecting all rings in order to separate the perfect and the discard rings. So that the perfect rings must carry the entire manufacturing cost of both perfect and wasted rings additional to the cost of inspection. And with a fairly high waste ring factor present, the production cost of the piston ring department of an auto plant or of the plant manufacturing rings alone, requires a comparatively high selling price in order to cover the losses produced by the presence of the imperfections in the initial casting.

The general purpose of the present invention is to eliminate this loss by eliminating its source—the imperfections in the casting. And to produce this result I employ the general principles of adhesion. For instance, if a suitable structure be moved through the molten metal in the direction of natural flow of the imperfection sources, these latter will pass to and move with the

structure through the molten metal during movement of the structure. So that if the structure be located at the bottom of the mold and then be drawn through the molten metal toward the waste neck of the casting, the bubbles or the sand particles will be carried from the service portion of the casting and moved into the waste portion, if the structure move into the latter; if the structure be withdrawn the imperfection sources will be brought to the surface.

Obviously, the structure employed for removing the imperfection sources would have dimensions such as to be of less thickness than the thickness of the casting wall on the plane of action of the structure. For instance, if the casting be of cylinder form and comparatively thin-walled—the piston ring supply casting, for example—the structure may be in the form of a ring of wire of suitable material and gage and of a diameter such as to be approximate the medial diameter of the cylinder, so that, if accurately positioned, the ring would be substantially symmetrically positioned within the cavity of the mold and thus pass through the molten metal approximately central of the wall thickness. Accuracy to an extreme degree is not, however, required in the movement of the structure through the centre of the wall, approximate accuracy being sufficient, it being preferred that the structure move within the molten mass rather than in contact with the mold wall, since such latter movement might tend to increase the introduction of the sand particles.

One or more wire elements may be secured to the structure, these extending vertically and of a length to project above the mold cavity, these serving as handles to move the structure through the metal; and for convenience the ends of these handles may be bent laterally or otherwise shaped to permit ready manipulation of the structure.

The movement of the structure may be had upon completion of the pouring—if the wall thickness is such as to delay the beginning of solidification sufficiently to permit the pouring and the movement of the structure to be completed. However, a preferred way of use is to locate the structure at the bottom of the mold cavity and after a portion of the metal has been poured, begin the movement of the structure upwardly—in the direction of natural movement of the imperfection sources—and continue such movement during the remainder of the pouring movement, the active portion of the structure always remaining below the level of the poured metal; the structure thus “follows up” the level of the poured metal, and after pouring has been ended, the movement is continued until the active part of the structure has passed into the waste zone or entirely removed. If permitted to remain

in the waste zone of the casting, it becomes embedded therein through the solidification action and can be cast aside with the waste "neck," being serviceable as a handle for 5 the casting while so embedded.

It is to be understood, of course, that the movement of the eliminating structure takes place while the metal is molten so that free movement of the structure is had and movement of the imperfection sources can take place. Surface cooling probably does not affect the action as long as the sources are free to move with the freely moving eliminating structure. If the metal be in its fluid 10 or molten state, however, the movement of the structure will cause the imperfection sources to pass to it and move onward with it as long as the structure is embedded within the molten metal, doing this through the 15 activity of the general conditions of adhesion—and possibly some of the characteristics of adsorption—the shifting of the molten metal by the passage of the structure through it aiding in this result, the metal 20 closing in behind the advancing structure and forming a casting from which the imperfection sources have been removed.

By the elimination of the source of the imperfections the casting becomes wholly 25 serviceable, so that wastage in rings is prevented, and it becomes practically unnecessary to provide inspection of rings, where the methods are employed in the production 30 of piston-ring-supply castings.

To these and other ends, therefore, the nature of which will be readily understood as 35 the invention is hereinafter disclosed, said invention consists in the methods of casting hereinafter more fully described, illustrated 40 in the accompanying drawings, and more particularly pointed out in the appended claims.

In the accompanying drawings, in which similar reference characters indicate similar parts in each of the views,—

Figure 1 is a vertical central sectional view of a mold for producing the blank cylinder which forms the supply for the production of piston rings, showing the 50 elimination structure in initial position.

Fig. 2 is a similar view of the upper end of the mold, showing the elimination structure raised to the waste zone and frozen into the material of the zone.

Fig. 3 is a perspective view of one form of 55 elimination structure that may be employed.

Fig. 4 is a similar view of a different formation of the elimination structure.

Fig. 5 is a sectional view of a portion of a 60 mold showing another way in which the invention may be practiced.

As heretofore pointed out, I have shown the invention as employed in connection with the casting of the cylinder that forms the 65 supply source for the production of piston

rings, a form that presents the characteristics of a circular tube. It is obvious that the casting to be formed may be of other cross-sectional contour, so that it is unnecessary to show other forms, that shown being 70 sufficiently illustrative to enable a proper understanding of the characteristics of the invention to be had.

In the drawing, the mold—shown as a sand mold for purpose of illustration—is indicated at 10, and the core at 11, these being arranged to form a cylindrical cavity 11 with an enlarged "neck" 11<sup>a</sup>, the latter receiving the material of the waste zone of the casting. As the mold is shown as having the top of the cavity closed, it will be understood that the usual pouring gate will be employed; obviously, however, the mold may have its top open. As will be understood, the length of the cavity 11 will be that required to produce the desired length of supply cylinder—the general standard being about eight inches, while the thickness of the wall of the cylinder casting will be such as to provide the proper size ring when the 85 casting has been machined.

Because of the comparatively thin wall of the cylinder, it will be readily understood that the inner and outer surfaces of the poured metal cool rapidly, so that the casting 95 is of a rapid solidification characteristic. This, as previously pointed out, sets up the conditions of imprisoned gas bubbles and of sand particles, solidification taking place before these can pass to the top waste 100 zone through the natural action. It is to meet this condition, and aid in the elimination through producing a rapid movement of an elimination structure or instrumentality through the molten metal in the general 105 direction of the natural movement of the imperfection sources, thus carrying these to the waste zone before solidification takes place.

The elimination instrumentality may be 110 of any suitable form and material, two simple forms—applicable for use in the particular mold of the drawings—being illustrated as examples of what may be used for the purpose. Each of these sets up the conditions of a portion that has the general contour of a cross-section of the supply portion of the casting, and a portion or portion that may serve as handles to this portion.

Since the contour of the cavity shown in 120 the drawing is circular, the portion 12 of the instrumentality has this contour, either by being of a substantially continuous ring contour, as in Fig. 3, or by the use of two segmental portions 12<sup>a</sup> adapted to be placed in 125 position to set up the ring-shaped contour, as in Fig. 4. In either case, the cross-section of the material of the ring or segment is sufficiently less than the width of the cavity as to ensure that it can travel through the mol- 130

ten metal without disturbing the surface of the poured metal at the sides of the positioned metal, the purpose being to prevent action such as scraping of the cavity walls or raising the metal within the cavity, but permitting free movement through the molten metal.

At the commencement of the pouring the ring-shaped portion of the instrumentality will be properly positioned at the bottom of the cavity, and to permit its manipulation a suitable handle portion 13 is attached to the ring portion, this handle portion being shown as a pair of rod-like portions of sufficient length to project from the top of the mold, this being simply illustrative of various forms and positions of handles that may be employed. The handles are shown as oppositely-disposed and may, if desired, be bent laterally or given other formations external of the mold to enable the workman to more readily manipulate the instrumentality.

The instrumentality may be formed of wire of suitable material. It may be of the material of which the casting is made so that should there be any tendency to be melted, it will not affect the material of the casting; preferably it is of material of sufficient heat resisting quality to maintain itself during the short period it remains within the cylinder portion of the mold.

The handles may be secured to the ring-shaped portion in suitable manner, as by welding, but preferably by being integral with it; and for purposes of ready production, but one handle may be provided, although I prefer to use at least two, since this permits of more accurate raising of the ring through the molten metal. Possibly a simpler and less expensive formation is illustrated in Fig. 4, in which the instrumentality is of two parts, each having a pair of handles, the assembly of the two parts placing two handles—one from each part—side by side. Obviously, other ways or forms may be employed for producing the instrumentality, as, for instance, one of the handles of the segment of Fig. 4 may be omitted, and the free end of the segment united to the handle of the other segment. And it will be understood that, in practicing the invention, the double member instrumentality would be operated in the same manner as the single member structure of Fig. 3, both members being moved upwardly concurrently.

The instrumentality may "follow" the level of the exposed surface during pouring, or the movement of the instrumentality may be delayed until the pouring has been completed, this depending more or less upon the time that elapses between pouring of the metal and its solidification to such an extent as to prevent the desired action of the instru-

mentality. The particular conditions present in the production of the casting will determine which course to pursue. Where the action is that of "following up" the top surface of the poured metal, it is necessary that the ring portion remain below the surface.

As heretofore pointed out, the movement of the instrumentality through the molten metal sets up the conditions of the principles of adhesion, the air or gas bubbles, or the sand particles, moving to the ring part and rising with the latter, thus moving at a different speed from the natural speed of travel of these imperfection sources in a casting of this type, the instrumentality thus aiding the elimination of these sources by changing the speed of travel from the natural speed to that of the instrumentality itself. So that, if the speed of travel of the instrumentality be sufficiently rapid as to permit it to reach the waste zone of the casting before actual solidification is set up, the imperfection sources will be carried to this zone and the supply portion of the casting will be freed of these imperfections.

The instrumentality may be permitted to "freeze" within the waste zone of the casting, and thus serve as a handle for the casting; this is especially the case where the mold carries a top, the latter then carrying suitable openings through which the handles extend and are moved. Where an open top mold is employed, the instrumentality may be entirely withdrawn, leaving the imperfection sources within the waste zone; but inasmuch as the instrumentality will possibly become useless after performing the service, there is probably no advantage to be gained through entirely withdrawing it.

As will be understood, the instrumentality can be positioned within the cavity at the time the mold is produced, remaining there until the pouring of the metal takes place.

If desired, the surface of the instrumentality may be provided with a coating; for instance a coating of clay may be applied and baked thereon, thus rendering the metal of the instrumentality less likely to be affected by the heat of the molten metal.

As will be understood, the portion of the instrumentality that is mainly effective in practicing the invention is the ring-like portion shown in the drawing—that portion that corresponds in contour to the cross-section of the casting; the handle portion is designed more particularly for the purpose of moving the ring. Because of this fact it is possible to vary the particular method of providing the ring movements, an additional way being shown in Fig. 5, in which the ring is free from connection with handles and is moved by members 15 that are movable through the lower wall of the mold, these members resting flush with the bottom of the cavity, and being moved upward.

ly to raise the ring into the waste portion of the casting and then quickly withdrawn to the initial position to maintain the bottom of the cavity closed. Members 15 may be 5 separate wires, or may form a part of an instrumentality fabricated to permit of concurrent movement—cross-head 15<sup>a</sup> illustrating a simple arrangement for the purpose. This way of practicing the invention 10 may be advantageous under certain conditions, but necessitates that the movement of the ring be completed while the metal remains sufficiently fluid to permit withdrawal of the members 15 before solidification and 15 in order that the metal of the casting may flow into the space left vacant by the members.

As will be understood, the method herein set forth is more particularly adapted for 20 service under conditions where the casting is of a comparatively thin-walled type, thus permitting the action of the instrumentality to become effective without materially disturbing the molten metal itself as the instrumentality moves through it, a result permitted by the use of an instrumentality of 25 comparatively small cross-sectional dimensions and at the same time be effective in setting up the conditions of adhesion reaching substantially to the surface of the casting. Where the casting is of thick walls or 30 is of solid formation, as with billets, etc., for instance, the effective zone of adhesion can only reach the surface by the use of an instrumentality of relatively large cross-sectional 35 dimensions, the result being that there is a material disturbance of the molten metal by the instrumentality during the withdrawal activity, due to the necessity of the 40 metal above the instrumentality to pass around the latter, an action that could readily produce gas bubble formations as well as dislodge sand particles from the mold, leaving the casting with the imperfections present 45 therein. Hence, in referring to "thin-walled structures" it is the intention to place in somewhat contrasting effect, the type of structures referred to herein and those which may be of the billet or the ingot type, or of 50 structures of solid formation having relatively large dimensions, such latter structures having dimensions such as to render it difficult, if not impracticable, to eliminate imperfections by the methods herein described, due to the fact that the large cross-section would require at best a very complicated instrumentality, the use of which 55 would set up other difficulties such as to make the use of the method less advantageous.

While I have herein shown and described several ways in which the general invention may be practiced, as well as different forms of instrumentalities that may be employed 60 therein, it will be readily understood that

these are simply illustrative and that variations and modifications in the methods and in the instrumentalities employed may be found desirable or essential in meeting the various exigencies of use; for instance, the 70 mold may be of other materials than sand—a metal mold, for example. I therefore desire to be understood as reserving the right to so vary or modify the methods practiced and the instrumentalities employed in such 75 practice, as may be found desirable or necessary, in so far as such variations or modifications may fall within the spirit and scope of the invention as expressed in the accompanying claims, when broadly construed.

Having thus described my invention, what I claim as new is:

1. In the art of casting metal for the production of castings of generally uniform 85 cross-section in the direction of length of the casting, and wherein the casting is of a comparatively thin-walled type, the method of eliminating imperfections of the bubble or hole type therefrom, which method consists in moving the imperfection sources from the poured metal to a waste zone by increasing the normal speed of travel of the sources in the direction of natural movement thereof to an extent sufficient to carry the sources 90 to such zone prior to solidification of the metal.

2. In the art of casting metal for the production of castings of generally uniform cross-section in the direction of length of 100 the casting, and wherein the casting is of a comparatively thin-walled type, the method of eliminating imperfections of the bubble or hole type therefrom, which method consists in moving the imperfection sources 105 from the poured metal to a waste zone by moving an instrumentality bodily through the poured metal in the general direction of natural movement of the imperfection sources and intermediate and spaced from 110 the faces of the casting and throughout the source zone of the casting, the movement of the instrumentality being at sufficient speed as to complete its movement to the waste zone prior to metal solidification to thereby 115 cause the imperfection sources to pass to and be carried with the instrumentality by adhesion.

3. In the art of casting metal for the production of castings of generally uniform 120 cross-section in the direction of length of the casting, and wherein the casting is of a comparatively thin-walled type, the method of eliminating imperfections of the bubble or hole type therefrom, which method consists 125 in moving the imperfection sources from the poured metal to a waste zone by locating an instrumentality of the general configuration of a cross-section of the casting and of less dimensions than the thickness of the casting 130

6

wall at the bottom of the mold in advance of pouring the metal, and then moving such instrumentality bodily through the poured metal toward and into the waste zone of the casting prior to solidification of the metal to thereby present movement of a body through the intermediate portion of the molten metal in the direction of natural movement of the imperfection sources to cause such sources to pass to and be carried by the body into the waste zone at a speed greater than the natural speed of travel of the sources.

4. In the art of producing castings of circular contour and adapted to form the supply for the production of piston rings, and wherein the casting includes a waste zone located at the upper end of the casting when being produced, the method of eliminating imperfections of the bubble or hole type from the casting, which method consists in locating an instrumentality at the bottom of the mold and between and spaced from the opposing walls of the mold cavity with the instrumentality contour of a form to correspond generally to a cross-section of the casting ring-supply portion, and then moving the instrumentality through the poured metal in the direction of natural movement of the imperfection sources and toward and into the waste zone prior to metal solidification, the movement of the instrumentality causing the imperfection sources to pass to and be carried with the instrumentality by adhesion activity into the

waste zone at greater speed than the natural speed of travel of such sources through the molten metal.

5. In the art of casting metal for the production of castings of generally uniform cross-section in the direction of length of the casting, means operative by its movement through the molten metal of the casting in the direction of natural movement of imperfection sources to a waste zone to eliminate imperfections of the bubble or hole type from the casting, said means including an instrumentality having a contour in general correspondence with the contour of a cross section of the casting and having dimensions such as to be less than the distance between the opposing walls of the mold cavity to permit location thereof intermediate and spaced from such walls, and means operative to move the instrumentality bodily through the poured metal to carry the instrumentality into the waste zone in advance of metal solidification.

6. Means for moving the instrumentality as in claim 5 characterised in that the instrumentality-moving means is adapted to cause instrumentality movement in a direction substantially parallel to the walls of the mold cavity to retain the instrumentality within the molten metal and spaced from the opposing surfaces thereof.

In testimony whereof I have hereunto affixed my signature.

JAMES M. PERRY.